

Oct. 19, 1954

M. D. WHITNEY

2,692,198

METHODS OF PRODUCING HALF-TONE PRINTING PLATES

Filed Aug. 11, 1950

2 Sheets-Sheet 1



INVENTOR.  
MAURICE D. WHITNEY  
BY

*Maurice D. Whitney*  
ATTORNEY

Oct. 19, 1954

M. D. WHITNEY

2,692,198

METHODS OF PRODUCING HALF-TONE PRINTING PLATES

Filed Aug. 11, 1950

2 Sheets-Sheet 2



INVENTOR.  
MAURICE D. WHITNEY  
BY

  
ATTORNEY

## UNITED STATES PATENT OFFICE

2,692,198

## METHODS OF PRODUCING HALF-TONE PRINTING PLATES

Maurice D. Whitney, Rocky Ford, Colo.

Application August 11, 1950, Serial No. 178,810

4 Claims. (Cl. 95—5.6)

1

This invention relates to a method and means for producing printing plates for use in printing pictorial illustrations upon conventional printing presses.

The principal object of the invention is to provide a method and means whereby the usual acid-etched metallic plates and the steps involved in their manufacture will be eliminated so that the process may be used by small town newspapers and other printing establishments not having the present engraving facilities available.

With the usual acid-etched plates, the depth of etch decreases as the fineness of the screen increases. This decreases the height of the printing protuberances so greatly that fine screen engravings cannot be satisfactorily used on soft papers. Another object of this invention is to produce a printing plate which will have a uniform "depth of etch" at all screen meshes.

Other objects and advantages reside in the detail construction of the invention, which is designed for simplicity, economy, and efficiency. These will become more apparent from the following description.

In the following detailed description of the invention, reference is had to the accompanying drawing which forms a part hereof. Like numerals refer to like parts in all views of the drawing and throughout the description.

In the drawing:

Fig. 1 is an illustration of a photographic negative from which the improved printing plate is to be produced;

Fig. 2 is a magnified view of a screen employed in the process;

Fig. 3 illustrates a sheet of transparent plastic material employed in the improved process;

Fig. 4 illustrates a plastic sheet carrying a photographic light-sensitive emulsion which forms the final printing plate in the process;

Fig. 5 is a greatly magnified enlargement of a portion of the screen of Fig. 2;

Fig. 6 is an enlarged cross-section illustrating the plate of Fig. 4, with the transparent plastic sheet of Fig. 3, the screen of Fig. 2, and the negative of Fig. 1 superimposed thereon;

Fig. 7 is a greatly magnified view of a portion of printed matter which is finally produced from the negative of Fig. 1;

Fig. 8 is a still further magnified view of a portion of the matter of Fig. 7;

Fig. 9 illustrates the completed emulsion plate mounted on a backing block for use in the printing press; and

Fig. 10 is a diagrammatic view illustrating the use of a photographic enlarger in the improved process.

In Fig. 5 lines have been used to designate var-

2

iations in opaqueness. In the actual screen the variations would be in density only.

The general method of reproducing photographic pictures in newspapers and the like consists of the following steps: (1) exposing a photographic film in a press camera; (2) making a photographic print of the film; (3) re-photographing the photographic print through a line screen to produce a negative film of the picture in dots through the interstices of the screen; (4) photographically printing this screened negative on a metal plate having a light-sensitive emulsion to form a screened positive on the plate; and (5) immersing the screened positive plate, after development, in acid to etch away the unexposed portions of the plate face to produce the final printing plate.

The improved process eliminates steps 2, 3 and 5, that is, the original print, the screened negative and the acid etching are no longer required, and a printing plate is produced directly from the image formed on the original negative in the press camera. In the improved process only the original press camera negative, diagrammatically indicated at 10, and a flexible final printing plate, indicated at 11, are produced. There is some loss of pictorial quality each time an image is reproduced from one photographic material to another. By eliminating the image transfer from camera negative to photographic print and from this print to a line screen negative much more of the original quality of the image is retained by the use of the process herein outlined.

The final printing plate consists of a sheet of synthetic resin or other flexible plastic material. One surface of the plate 11 is coated with a relatively heavy, photographic, light-sensitive emulsion 12 to which a reversed positive image of the negative 10 is transferred through a screen 14 and through a transparent plastic sheet 13.

The positive image on the emulsion 12 is then developed, treated, and hardened. The treatment of the emulsion causes the portions thereof which have not been exposed to light to be lowered and the portions which have been exposed to be raised above the normal emulsion surface to produce the final printing plate 11. Only the raised light-exposed portions of the plate will contact the inking rollers of the press and the paper upon which the picture is to be printed.

The usual line screen consists of a series of opaque crossed lines, the lines being of uniform density throughout their widths. The improved screen 14, however, consists of a series of crossed lines of varying density throughout their widths, as shown in the magnified view of Fig. 5. Each line consists of a completely opaque medial line

16 bordered at both sides with portions 17 of varying density. The variable density borders 17 on the lines 16 shade out gradually from the completely opaque line 16 to substantially transparent edges which border transparent interstices or open spaces 18. The complete width of the variable density lines, including portion 16 and both portions 17, is substantially equal to the width of the interstices 18. The center to center spacing of the lines is uniform in both directions and can conform to the various meshes of the standard photo-engraver's screens. For most uses the lines will be spaced 125 per inch.

The plate 11 is formed from a relatively heavy, cellulose acetate sheet having a thickness of at least 0.0073 inch. The emulsion 12 on the acetate sheet has a thickness of from 0.0009 inch to 0.004 inch, and the light-sensitive portion of the emulsion is of any suitable variety having high contrast, high resolving power, and fine grain. The plate 11 has a thicker emulsion coating and the coating has a greater silver salt content than the usual photographic emulsion in order to give a greater thickness or depth to the final printing surface, and greater height to the exposed dot formation which is finally formed thereon.

In the simplest form of the improved process, the plate 11 is placed upon a flat supporting surface, preferably a vacuum plate, as shown at 19 in Fig. 10, with its emulsion face upward. The screen 14 is placed over and tightly against the emulsion 12 and, for direct contact work, the camera negative 10 is placed over the screen 14, as shown in Fig. 6 and exposed to a suitable printing light. Preferably and usually, however, the negative 10 is placed in a photographic enlarger, as shown at 20 in Fig. 10, and the image is projected onto the emulsion 12 through the screen 14. In either case, the negative is inverted so that its emulsion side faces upwardly in order to effect lateral reversal of the image on the printing plate and the exposed emulsion 12 is then treated as will be later described.

In the preferred form of the process, the sheet 13 of clear plastic is placed between the screen 14 and the emulsion face 12 of the plate 11 before the exposure is made either by direct contact printing, as shown in Fig. 6, or by means of the enlarger projection, as shown in Fig. 10. The sheet 13 is allowed to remain in place for approximately one-sixth of the total exposure time. The transparent plastic sheet is then removed and the exposure is completed with the screen 14 in tight contact with the emulsion 12. Any desired means may be employed for holding the screen in register with the exposed emulsion 12. The vacuum plate 19 has been found satisfactory for this purpose.

After exposure, the plate 11 with its exposed emulsion is developed in an extremely high contrast developing solution, preferably having the following formula:

|                      | Oz.   |
|----------------------|-------|
| Water                | 24    |
| Sodium sulfite       | 3     |
| Hydroquinone         | 1 1/2 |
| Sodium hydroxide     | 1 1/4 |
| Potassium bromide    | 1     |
| Water to make 32 oz. | 70    |

The developed emulsion is then fixed in the usual hypo-fixing bath to set the exposed silver and dissolve out the unexposed silver to cause a resulting shrinking of the unexposed por-

tions of the emulsion. After washing, the emulsion is treated in a solution, preferably having the following formula:

|                         | Oz. |
|-------------------------|-----|
| Potassium bichromate    | 3   |
| Hydrochloric acid       | 2   |
| Water to make 1 gallon. |     |

This causes further shrinkage of the unexposed portions of the emulsion from which the silver has been dissolved and an expansion of the silver containing exposed portions thereof.

After a second washing the rough, indented surface of the emulsion is hardened by any suitable hardening solution, such as a solution consisting of:

|                  |       |      |
|------------------|-------|------|
| Iodine           | grams | 50   |
| Potassium iodide | do    | 100  |
| Water            | cc.   | 1000 |

The completed, hardened printing plate is then cemented or tacked to a wooden or metal backing block 15 which is used in the printing press in the same manner as the usual zinc or copper etching.

The final printing surface consists of a multiplicity of projections or "dots." With the screen illustrated, these dots will be quadrangular in shape and of varying surface area corresponding to the variations in light and shade in the original negative 10. For instance, the letters illustrated on the negative of Fig. 1 are transparent at their tops and become increasingly opaque as their bottoms are approached. It will be seen from the magnified view in Fig. 7 that in the final printing from the plate 11, produced from the negative 10, the quadrangular dots are relatively large and close together at the tops of the letters and diminish in size as the bottoms are approached.

The above results from the fact that the more intense light passing through the more transparent portions of the negative can penetrate further into the variable density borders 17 of the screen 14. Thus, the width of the dots is in direct proportion to the intensity of the light striking the screen which, of course, will produce the final half-tone shading on the printed piece.

It is desired to call attention to the fact that the size of the final dots may also be regulated by the use of the plastic sheet 13. The thickness of this sheet controls its effect on the dot sizes. If the sheet 13 were exceedingly thin or eliminated entirely, the dots in the shadow areas would approximate the open spaces in the screen and this has been found to produce a "flat" image with very little contrast. A transparent sheet having a thickness of 0.02 inch causes the dots to run together to produce a muddy, unsatisfactory plate. It has been found that if the sheet 13 has a thickness of from .003 to .013 inch the light from the printing lamp will spread after it passes through the interstices in the screen to produce larger dots on the emulsion separated by clear narrow lines which greatly increase the contrast of the final printing by creating deeper black in the dark areas. Therefore, the sheet 13 and its thickness and the control of its time of use during the exposure are the important control features of the invention. The short exposure with the plastic sheet 13 in place produces a larger and more solid dot structure for the shadow portion of the image on the emulsion 12 with the loss of detail in the lighter portions of the camera negative 10. The longer exposure of the image with

the screen 14 in direct contact with the emulsion 12, however, produces the high light detail. Variations of the total exposure and the ratio of exposure, with or without the plastic sheet 13 is used to control both contrast and total density in the emulsion 12.

While a specific form of the improvement has been described and illustrated herein, it is desired to be understood that the same may be varied, within the scope of the appended claims, without departing from the spirit of the invention.

Having thus described the invention, what is claimed and desired secured by Letters Patent is:

1. A method of producing a printing plate from a photographic negative of a picture, for use in a printing press, comprising: placing a transparent spacing sheet over a light-sensitive gelatin silver salt emulsion carried by a backing plate, placing a varying density halftone screen over said transparent spacing sheet, placing said negative over said screen, passing light through the superimposed negative, screen, and spacing sheet to expose said light-sensitive emulsion, then removing said sheet and completing the exposure with the screen in contact with said emulsion, developing the exposed positive emulsion to produce a positive image of said negative thereon, thence dissolving away the unexposed light-sensitive salts from said emulsion to cause a shrinkage of the latter in correspondence with the varying densities of said image, treating with acid bichromate solution for shrinking those portions of the gelatin from which the unexposed salts have been dissolved to produce an indented printing surface on said backing sheet, then hardening the emulsion by treating the same with a

solution of potassium iodide and iodine, and thence applying printing ink to the protuberances of said surface, so that said ink will offset against a sheet brought into contact with said surface.

5 2. The method according to claim 1 wherein said varying density halftone screen consists of a series of intersecting lines of varying density throughout their widths.

3. The method according to claim 1, wherein 10 said acid bichromate solution comprises a proportion of 3 oz. potassium bichromate, 2 oz. hydrochloric acid, and water of a volume to make 1 gallon in all.

4. The method according to claim 1, wherein 15 said hardening solution comprises a proportion of 50 grams iodine, 100 grams potassium iodide, and 1000 c.c. of water.

#### References Cited in the file of this patent

#### UNITED STATES PATENTS

| Number       | Name             | Date           |
|--------------|------------------|----------------|
| 381,091      | Sutton -----     | Apr. 10, 1888  |
| 878,505      | Cochran -----    | Feb. 11, 1908  |
| 1,354,001    | Fifer -----      | Sept. 28, 1920 |
| 25 1,464,139 | Ruhland -----    | Aug. 7, 1923   |
| 1,793,070    | Eldridge -----   | Feb. 17, 1931  |
| 2,150,805    | Meulendyke ----- | Mar. 14, 1939  |
| 2,244,187    | Cochran -----    | June 3, 1941   |
| 30 2,384,857 | Terry -----      | Sept. 18, 1945 |
| 2,405,291    | Corbett -----    | Aug. 6, 1946   |
| 2,533,650    | Wattier -----    | Dec. 12, 1950  |

#### FOREIGN PATENTS

| Number   | Country             | Date         |
|----------|---------------------|--------------|
| 35 5,008 | Great Britain ----- | of 1892      |
| 168,578  | Great Britain ----- | June 1, 1922 |